

## UNITED STATES PATENT OFFICE

2,221,259

## MAGNESIUM BASE ALLOY

John C. McDonald, Midland, Mich., assignor to  
The Dow Chemical Company, Midland, Mich.,  
a corporation of Michigan

No Drawing. Application November 13, 1939,  
Serial No. 304,136

3 Claims. (Cl. 75—168)

The invention relates to magnesium base alloys. It more particularly concerns alloys of this nature having a high degree of formability coupled with other improved physical properties, such as improved strength characteristics.

Magnesium alloys are enjoying increasing use in the structural and mechanical arts where a light weight metal is highly desirable, such as for use in making large castings, forgings, and the like. However, the use of these alloys in the rolled form to make sheet metal articles requiring forming operations has not progressed as rapidly due to the fact that in general alloys of good formability, permitting relatively sharp bends to be made without the article developing external cracks, usually have inferior characteristics as regards their tensile and yield strengths.

It is, accordingly, the principal object of the invention to provide a magnesium base alloy which may be made into rolled sheet or the like, possessing a sufficient degree of ductility or formability to be sharply bent, drawn, or otherwise shaped, while having improved tensile and yield strengths.

Other objects and advantages will be apparent as the description of the invention proceeds.

My invention resides in the discovery that a magnesium base alloy composed of from 0.3 to

coupled with high tensile and yield strengths, is found in alloys containing from 0.5 to 5 per cent of silver, 0.1 to 0.3 per cent of calcium, 5 to 10 per cent of cadmium, 1.5 to 2.5 per cent of manganese, and from 0.5 to 5 per cent of zinc.

The specific proportions of each alloying metal and the total amount of added alloying metals to be employed depends upon the use for which the alloy is intended. In general it is preferable to employ an alloy containing more than about 75 per cent of magnesium and less than about 25 per cent of the total added alloying metals. For example, in alloys where a high ductility or formability is of prime importance, the total added alloying metals should not exceed about 15 per cent, while in those instances where high yield and tensile strengths are desired, especially in the cold-rolled state, higher percentages of the alloying metals should be employed.

The following table, which lists some of the properties of rolled sheet metal made from my new alloys, as well as the properties of the related parent alloys in similar form, illustrates the improvement in yield and tensile strengths, and ductility or formability of the new alloys over that of the closely related alloys. In the table, the per cent elongation represents the ductility or formability of the alloys.

| 30 | Nominal composition in percent<br>(magnesium—remainder) |     |     |     |     | Annealed                             |                                        |                                      | Cold rolled                          |                                        | 30 |
|----|---------------------------------------------------------|-----|-----|-----|-----|--------------------------------------|----------------------------------------|--------------------------------------|--------------------------------------|----------------------------------------|----|
|    | Ag                                                      | Ca  | Cd  | Mn  | Zn  | Yield<br>strength in<br>lbs./sq. in. | Tensile<br>strength in<br>lbs./sq. in. | Percent<br>elongation in<br>2 inches | Yield<br>strength in<br>lbs./sq. in. | Tensile<br>strength in<br>lbs./sq. in. |    |
| 35 | 0.9                                                     | 0.3 | 5.2 | 1.1 | 4.7 | 22,000                               | 39,000                                 | 15                                   | 43,000                               | 48,000                                 | 35 |
|    | 1.0                                                     | 0.3 | 5.8 | 1.4 | 4.5 | 24,000                               | 37,000                                 | 16                                   | 39,000                               | 45,000                                 |    |
|    | 0.9                                                     | 0.3 | 2.8 | 1.4 | 4.5 | 31,000                               | 45,000                                 | 14                                   | 45,000                               | 52,000                                 |    |
|    | 0.9                                                     | 0.3 | 7.9 | 1.7 | 0.8 | 25,000                               | 39,000                                 | 16                                   | 42,000                               | 48,000                                 |    |
| 40 | 1.0                                                     | 0.3 | 8.5 | 2.1 | 0.9 | 25,000                               | 39,000                                 | 18                                   | 40,000                               | 45,000                                 | 40 |
|    | 1.0                                                     | 0.3 | 2.8 | 0.9 | 0.9 | 28,000                               | 40,000                                 | 16                                   | 41,000                               | 49,000                                 |    |
|    | 0.8                                                     | 0.3 | 9.2 | 0.8 | 0.8 | 20,000                               | 33,000                                 | 21                                   | 38,000                               | 44,000                                 |    |
|    | 0.7                                                     | 0.3 | 8.9 | 1.3 | 0.8 | 26,000                               | 32,000                                 | 18                                   | 41,000                               | 48,000                                 |    |
|    | 0.9                                                     | 0.3 | 8.2 | 2.0 | 0.8 | 30,000                               | 41,000                                 | 17                                   | 44,000                               | 51,000                                 |    |
|    | 5.2                                                     | 0.3 | 5.0 | 1.5 | 0.9 | 24,000                               | 40,000                                 | 16                                   | 47,000                               | 52,000                                 |    |
|    | 5.5                                                     | 0.3 | 4.9 | 1.8 | 0.9 | 27,000                               | 43,000                                 | 19                                   | 48,000                               | 54,000                                 |    |

45 10 per cent of silver, 1 to 15 per cent of cadmium, 0.05 to 1.0 per cent of calcium, 0.1 to 3 per cent of manganese, and from 0.1 to 10 per cent of zinc, the balance being substantially all magnesium, is endowed with the afore-mentioned properties. While the property of satisfactory formability or ductility, coupled with high tensile and yield strengths, is manifest over the entire range of composition indicated, I have found that in general the preferred combination of properties, 50 such as good ductility for forming operations

45 The properties listed in the above table under the section headed by the term annealed were obtained by first rolling the alloys at a temperature between about 500° to 600° F., and thereafter annealing them at various temperatures through a temperature range of from 400° to 800° 50 F. The properties selected for the table were those of the annealed specimens which exhibited the maximum elongation. The properties listed under the section headed cold rolled were obtained by subjecting specimens of the alloys 55

which had been hot rolled at a temperature of from 500° to 600° F. to additional rolling in the cold state to bring about a total reduction of from 2 to 10 per cent. The properties selected 5 for the table were those of the cold rolled specimens which showed the greatest tensile and yield strengths, while having at least a 1 per cent elongation in 2 inches.

By comparison of the properties listed in the 10 above table, it will be observed that the combined properties of my new polynary alloys are superior to those of the parent alloys having somewhat similar percentages of alloying ingredients. For example, it will be noted that the 15 per cent elongation, which serves as a measure of the ductility, is satisfactorily high, while the yield strength and tensile strength in both the annealed and in the cold rolled state show marked improvement over that of the related 20 alloys. Similarly other portions of the composition range show improved properties over those of the related alloys.

While the new alloy is most useful in wrought 25 form, such as sheets, due to its formability characteristics, it may also be suitably used in making castings, forgings, extruded forms, and the like. It is further pointed out that my new alloy is amenable to solution and precipitation heat 30 treatments, which, accordingly, modify its properties.

The new alloy may be compounded in any of

the ways known to the art, such as by adding the alloying ingredients to the molten magnesium under a suitable flux. The flux should be substantially free from magnesium chloride if the calcium content of the alloy is to be above 0.3 5 per cent. In those instances where an alloy is to be compounded containing less than 0.3 per cent of calcium, the presence of a small amount of magnesium chloride in the flux does not exert an undue deleterious effect, but in this case it is 10 usually preferable to add the calcium last and without too much stirring, in order that the loss of calcium into the flux will be prevented.

I claim:

1. A magnesium base alloy containing from 0.3 15 to 10 per cent of silver, 0.05 to 1 per cent of calcium, 1 to 15 per cent of cadmium, 0.1 to 3 per cent of manganese, and from 0.1 to 10 per cent of zinc, the balance being magnesium.

2. A magnesium base alloy containing from 1 20 to 8 per cent of silver, 0.1 to 0.8 per cent of calcium, 1 to 12 per cent of cadmium, 0.1 to 3 per cent of manganese, and from 0.1 to 10 per cent of zinc, the balance being magnesium.

3. A magnesium base alloy containing from 0.5 25 to 5 per cent of silver, 0.1 to 0.3 per cent of calcium, 5 to 10 per cent of cadmium, 1.5 to 2.5 per cent of manganese, and from 0.5 to 5 per cent of zinc, the balance being magnesium.

JOHN C. McDONALD.

30